

## UNITED STATES PATENT OFFICE

2,275,851

PROCESS FOR TREATING FABRICS AND  
LIKE MATERIALS TO PRODUCE EFFECTS  
THEREIN AND PRODUCTS THEREFROMGeorges Heberlein and Ernst Weiss, Wattwil,  
Switzerland, assignors to Heberlein Patent Cor-  
poration, New York, N. Y., a corporation of  
New YorkNo Drawing. Application January 26, 1939, Se-  
rial No. 252,938. In Germany February 15,  
1935

## 10 Claims. (Cl. 8—114.5)

This invention relates to a process for pro-  
ducing pattern fabrics and products therefrom.

This application is a continuation-in-part of  
our copending application Serial No. 63,808, filed  
February 13, 1936, now Patent No. 2,171,513.

One of the objects of the invention is to pro-  
vide simple and novel processes for the produc-  
tion of pattern crepe-effects, pattern translucent  
or transparent effects or for the production of  
a combination of both effects.

Another object of the invention is to provide  
special starting fabrics containing different kinds  
of yarns which enable the production of the de-  
sired finish effects. According to the invention  
the starting fabric contains at least two different  
sets or kinds of yarns, one set being of such  
character as to be substantially insensitive to  
swelling agents or inactive to which the other  
of the two sets of yarns is sensitive or active,  
so as to give or enhance the desired optical con-  
trast between the respective areas of the fabric  
consisting of the two sets of yarns. Another  
object of the invention is to provide products  
from such processes having novel and improved  
characteristics. Other objects will be in part  
obvious and in part pointed out hereinafter.

The invention comprises the novel products as  
well as the novel processes and steps of processes  
according to which such products are manufac-  
tured, the specific embodiments of which are de-  
scribed hereinafter by way of examples and in  
accordance with which we now prefer to practice  
the invention.

## DEFINITIONS

By "opened-up" yarns as herein mentioned, we  
mean vegetable yarns that have been cleansed  
by boiling, scouring, bleaching or the like, to the  
extent that all or substantially all of the natural  
incrustations are removed, so as to render said  
yarns sensitive to swelling agents.

By the term "raw vegetable yarns" or similar  
expressions as herein used, we mean vegetable  
yarns having all or a sufficient amount of their  
natural incrustations adhering to the fibers so  
as to render said fibers relatively insensitive to  
swelling agents, although the yarns may have  
been given mild cleansing or other treatments  
which do not materially remove their natural  
incrustations.

By the term "effect yarns" as hereinafter used,  
we mean yarns which as woven are not substan-  
tially sensitive to the swelling agents applied to  
the fabrics containing such yarns.

The following relates to the production of 53

crepe-like effects and translucent pattern effects  
and intermediate materials used therein em-  
ploying scoured yarns and yarns containing nat-  
ural incrustations.

5. 1. TREATED YARNS COMBINED WITH RAW-INCURSTED  
YARNS

## (a) Producing crepe-like effects by shrinkage

In order to produce crepe-like effects (Crepon)  
10 in loose condition, it has already been suggested  
to weave together mercerized and unmercerized  
cotton yarn and to treat such fabric with mer-  
cerizing liquor without tension. Thereby the  
unmercerized yarn shrinks while the mercerized  
15 yarn is supposed to remain unshortened so that  
undulated extensions and depressions are  
formed on the fabric. This old process produces  
very unsatisfactory results. These unsatisfac-  
tory results occur because the mercerized yarns  
20 are effected also by a second treatment with  
mercerizing lye.

In accordance with one aspect of the present  
invention it has now been found that improved  
25 effects can be obtained by the use of starting  
fabrics containing "opened-up" yarns and raw  
yarns of vegetable fibers to which the natural  
incrustations still adhere. Swelling agents hav-  
ing a shrinking effect known to the textile fin-  
30 isher are then caused to act on such fabric in  
accordance with the present invention so that  
the yarn previously treated contracts while the  
crude yarn remains substantially uncontracted.  
If a very pronounced crepe-like effect is to be  
35 obtained, it is preferable to use alkali lyes of  
mercerizing strength. In this way there is pro-  
duced a crepe-like effect which may take the  
most varied forms depending on the distribution  
in the fabric of the raw "effect" yarns, that is,  
40 the yarns which according to this part of our  
invention are present initially in the fabric as  
raw yarn containing the natural incrustations.  
For example, the raw yarn may be woven to  
form stripes, diamonds, etc. Also other fabrics  
45 can be finished in the same manner, for instance  
knitted goods, hosiery goods, printed goods, etc.  
which consist of previously treated and raw veg-  
etable yarns containing incrustations may be  
employed.

50 After shrinking the fabric can be further  
treated in any desired manner, namely by  
bleaching, dyeing, finishing or the like. In dye-  
ing, "tone in tone" effects can be obtained since  
the previously treated "opened-up" fiber has the  
property of consuming more dye than the raw

fiber. The expression "tone in tone" is intended to indicate the effect given by such a combination of dyed fibers possessing different shades of color.

If this process is combined with the usual reserve printing process, peculiar and manifold effects can be obtained. For example the fabric prepared in accordance with the invention from previously treated and raw incrusted cotton yarn is printed locally with a gum reserve (gummi reserve) and after drying, is mercerized in loose condition. The yarn, protected by the reserve remains unchanged so that these parts stand out as pattern effects.

The process is preferably employed with cotton containing fabrics, but the other natural vegetable fiber products can be used instead of cotton. It is important, however, in selecting for the "effect" yarns such natural vegetable fibrous material as contains the natural incrustations. The fabric may contain one kind of fiber alone or there may be an admixture of fibers, so long as some of the yarns are relatively insensitive to the swelling agent.

The following examples embody the present aspect of the invention as we now prefer to carry it out, but the invention is not to be restricted thereto except as indicated in the appended claims.

*Example 1.*—Cotton muslin, the base of which consists of yarn previously scoured and into which effect-yarns of raw cotton containing incrustations are woven in stripes, is impregnated with caustic soda solution of 37° Bé. at 10° C. for 3 seconds. The material is pressed and set aside at room temperature for three minutes in unstretched condition. Thereupon it is washed hot at about 85° C., acidified and bleached carefully in the usual manner. Finally it is dried in loose condition. The effect produced is shown by the wave-like projections of the effect-threads which impart to the fabric a crepe-like character.

*Example 2.*—Muslin woven from scoured cotton yarn and also containing as effect yarns individual raw cotton yarns containing incrustations woven into warp and filling in diamond shaped patterns is printed with a gum resist, for example gum arabic, locally. After the drying of the resist the fabric is mercerized without tension in accordance with Example 1, washed, whereby also the resist is removed, and finished. The resist parts are set off as patterns from the checkered pattern background.

(b) *Producing transparent and translucent effects*

It is known that stiffened more or less transparent effects can be produced on cellulose-containing fabrics by means of various parchmentizing swelling agents. If this process is employed on fabrics in which thick yarns have been incorporated in thin fabrics for the purpose of producing a pattern, for example yarns woven in stripes or rectangular form, or if the process is employed on fabrics embroidered in figures forming denser parts of the fabric, the resulting products obtained by this old process have an ugly appearance. The thick incorporated threads become hard and brittle and bring about an excessive stiffness of the entire surface of the fabric.

It has now been found in accordance with this aspect of the present invention that these difficulties may be avoided if fabrics are prepared which contain on the one hand previously treated

yarns, that is "opened" yarns as described above, and on the other hand yarns which are substantially insensitive to swelling agents, namely raw yarns to which natural incrustations still adhere.

5 It has been found that the latter yarns are not influenced by agents for producing the stiffened more or less transparent effects.

As swelling agents for the production of these effects, there may be employed for example sulphuric acid of over 50.5° Bé. in conjunction with mercerized yarn, that is, mercerized yarn may be woven with a raw natural incrusted yarn and this material treated to produce a transparent effect in the mercerized yarn but substantially

15 without producing such effect in the raw incrusted yarn. Caustic soda solution at low temperatures, approximately -10° C., may also be employed for the transparentizing treatment in conjunction with sulphuric acid treatment. Al-

20 ternate treatments with caustic soda followed by sulphuric acid of 50.5° Bé. or over, followed by another treatment with caustic soda of mercerizing strength in the well-known manner may also be employed for producing transparentizing

25 effect on cotton yarn which has been "opened-up," while the naturally incrusted yarn interwoven therewith remains substantially without change. Other reagents that may be used to give similar translucent effects, as is well-known,

30 are the following agents used alone: sulphuric acid, phosphoric acid, mixed acid (nitric and sulphuric acid), caustic soda solution which has been cooled down to about -10° C., zinc chloride, calcium thiocyanate, ammoniacal copper oxide

35 and others. These reagents are employed under conditions of time, temperature and concentration which are well-known in the art, for example as shown in U. S. Patents 1,265,082 and 1,395,472.

40 According to the present invention the fabrics which have been treated to produce the translucent or transparent effects can, if desired, be further treated in order to render the original raw yarns containing the natural incrustations

45 susceptible to further treatment. For instance they can be treated to render them more absorptive to dyestuffs. Such raw naturally incrusted yarns can also be "opened" up by bleaching or other opening up process described above.

50 After the opening up of these raw yarns, they then exist in a fabric which, at least in part, has been rendered more transparent or more translucent. This fabric can be treated with a shrinking agent such as caustic soda which 55 will cause these non-transparent yarns to shrink so that a wavy effect will appear on the surface of the fabric of the transparent or translucent fabric.

In addition various effects can be obtained if 60 the swelling agent for producing transparency or translucency is only caused to act locally on the fabrics by direct or resist printing. Pattern effects produced in this manner can be further changed by treating them again subsequently 65 with swelling agents having a shrinking action as for instance caustic soda solution by which crepe-like patterns are obtained.

In addition combinations of simultaneous or successive local action of transparentizing agents (or agents for producing translucency) and shrinking agents can be employed. In connection with this patterns can be printed alongside of each other or on top of each other.

The effects mentioned can be further enriched 75 by dyeing and color printing in any conceivable

manner. Depending on the dyestuff selected there can be obtained thereby multi-stage shadings of the different colors because of the different action of the dyestuffs on the fibers treated by the transparentizing, shrinking and other swelling agents.

The following are specific examples of embodiments of this aspect of the invention as we now prefer to practice it. The invention is not restricted thereto, however, except as indicated in the appended claims.

*Example 3.*—A cotton muslin fabric, the base of which consists of scoured cotton yarns containing woven stripes of coarse raw cotton effect yarns containing natural incrustations is treated with sulphuric acid of 53° Bé. at 12° C. for 8 seconds. Thereupon the acid is washed out, the fabric is mercerized with caustic soda solution of 28° Bé. at 15° C. The fabric is then bleached. The resultant product is a transparent fabric in which appears stripe effects, these stripes being the raw cotton effect yarns which have not been transparentized due to the protective coating of the incrustations. These stripes remain soft and their presence does not tend to render the fabric more brittle. They give an optical contrast in which because of their non-transparent character, they are set off from the transparent base.

*Example 4.*—A cotton muslin fabric, the base of which consists of scoured cotton yarns and also containing woven stripes of coarse raw cotton yarns, as effect yarns, containing natural incrustations is treated with a solution of 70 parts of zinc chloride in 30 parts of water at 100° C. during 20 seconds. The fabric is then washed with cold water and finished in a frame. A similar effect is obtained as described in Example 3.

*Example 5.*—A cotton muslin consisting of scoured yarns and raw yarns as effect yarns forming a suitable design is printed with a resist of gum arabic and dried. Then it is treated with sulfuric acid of 54° Bé. during 10 seconds at 8° C. Then it is washed thoroughly, whereby also the resist is removed, and then bleached and finished. The resist parts stand out as patterns from the transparent background which is traced through by opaque designs due to the raw yarns.

*Example 6.*—A starting fabric of cotton muslin as described in Example 3 is transparentized in the same way as is pointed out in this example. The fabric is then kier-boiled and bleached and dried in a frame. Afterwards it is treated with caustic soda solution according to Example 1. The raw threads opened up by kier-boiling now shrink whereupon the transparent parts which remain substantially unchanged by the alkali treatment, assume a wavelike appearance.

## 2. UNCOATED YARNS COMBINED WITH COATED YARNS

### (a) Producing crepe-like effects by shrinkage

In accordance with this aspect of the present invention it has been found that instead of the vegetable yarns containing natural incrustations, there may be substituted yarns which have already been subjected to prior treatment, for instance bleached, mercerized or dyed yarns, but which prior to manufacture into fabric have been made insensitive or inert to the action of the swelling agents. There are suitable for this purpose natural vegetable yarns and artificial yarns of various kinds as well as yarns of animal origin.

The yarns or rayon threads which have been subjected to any desired prior treatment may be

made insensitive to the action of the swelling agents in following manner:

1. Sizing with sizing agents for instance starch, gum, tragacanth gum and the like.
2. Impregnating with water-repellent agents, for instance a 6% emulsion of commercial paraffin or with an emulsion of higher fatty acid anhydrides and the like.
3. Impregnating with solutions of waxes and higher melting fats and hydrocarbons, for instance 10% beeswax in benzine; 10% Japan wax in benzine; 8% synthetic wax in benzine; rubber in benzol/toluol, chlorinated rubber in toluol, paraffin in benzine and the like.
- 10 4. Production of film-like or varnish-like coatings on the yarns by means of varnishes and resin-like substances, for instance cellulose esters, for example 15% nitrocellulose in alcohol and ethyl acetate, solution of dimethyl urea, acetyl cellulose in acetone, and the like.

The vegetable or animal yarns or rayon yarns which have been made insensitive to swelling agents by any of the above-described methods are now woven with previously treated "opened-up" yarns, that is, with yarns which are affected by swelling agents. Especially favorable results may be obtained with lustrous and dyed yarns which have been made insensitive in the manner indicated above. The completed fabrics are shrunk by means of swelling agents known to the textile finisher including those mentioned above for crepe-like effects under 1(a). After the washing out of the swelling agent the insensitizing material, depending on its nature, may either be removed or may remain in the fabric. In the latter case, if their presence for some particular purpose should prove objectionable they may be removed by a special process. In most cases, however, such subsequent treatment is not necessary.

40 10 The completed fabrics can be improved further by subsequent dyeing if desired. Such dyeing may be performed if desired before the insensitizing materials have been removed.

This process may be combined with the customary resist printing processes, briefly referred to above, to obtain manifold effects.

The following are examples of embodiments of the invention just described. The invention is not limited thereto except as indicated in the 50 appended claims:

*Example 7.*—A calico fabric, the base of which consists of scoured yarns and also containing as effect yarns woven stripes of mercerized cotton yarns which have been impregnated with a solution made up from 15 parts of nitrocellulose, 57 parts of ethyl acetate and 28 parts of ethyl alcohol is treated with caustic soda solution according to Example 1. Similar effects to those of Example 1 are obtained but the luster of the mercerized 55 effect threads imparts a good appearance to the finished fabric.

*Example 8.*—A cotton muslin which contains scoured cotton yarns and as effect yarns, cotton yarns which have been mercerized, dyed and impregnated with a solution of 10% beeswax in benzine, is treated according to Example 1. A special effect is obtained by means of the dyed effect 60 yarns.

*Example 9.*—A fabric containing cotton yarns 70 impregnated with a lacquer of 20% chlorinated rubber in toluene and grey cotton yarns is scoured and bleached. This treatment removes the natural incrustations from the grey cotton yarns. Thereafter it is treated with a caustic soda solution of 30° Bé. without tension at 15° C. during 75

3 minutes, delayed with hot water, scoured, washed out and finished as usual.

(b) *Producing transparent and translucent effects*

Fabrics containing sensitive uncoated and insensitive coated yarns prepared as in 2(a) above may also be treated with agents to produce areas of transparency or translucency along with some stiffening of the fabric. The swelling agents employed for producing these effects may be the same as those given under the title 1(b) above. The effects produced by the use of these insensitive yarns are similar to the effects described under 1(b) above. The following are specific examples of this part of the invention, it being understood that the invention is not restricted thereto, except as indicated in the appended claims.

*Example 10.*—A cotton muslin the base of which consists of scoured yarns and also containing effect yarns made insensitive to the action of parchmentizing agents by impregnation with an emulsion of paraffin (for example "Migasol" marketed by "Gesellschaft für chemische Industrie, Basel") is treated with sulfuric acid in the same way as described in Example 3. The effect yarns remain soft and give an optical contrast because of their non-transparent character.

*Example 11.*—A fabric containing cotton yarns impregnated with a lacquer of 20% chlorinated rubber in toluene and grey cotton yarns is scoured and bleached. This treatment removes the natural incrustations from the grey cotton yarns. Thereafter it is treated with sulfuric acid of 54° Bé. at 17° C. during 10 seconds, washed out and finished as usual.

In the above examples, it will be noted that various fabrics are treated, in some of which, as in Example 1, the statement is made that yarns are woven in stripes, and in Example 2, yarns are "woven into warp and filling." It will be understood from all of the above Examples 1-11, that the fabrics are woven in a well-known manner so that, as is customary, the warp yarns are crossed by yarns of filling, and vice versa.

The fabrics prepared from the yarn as hereinbefore described may be of any kind, as, for instance, woven, braided or knitted fabrics, and may contain both kinds of yarns, namely, inactive and active yarns in varying proportions. Either the inactive or active yarns may predominate as desired to give different effects.

The fabrics prepared in accordance with the invention include, it will be observed, both shrunk crepe effects and transparentized effects. The shrunk effects include yarns woven in a pattern and which are unswollen, crossed by yarns which are swollen throughout the full length of the yarns. The transparentized effect fabrics include yarns woven in a pattern of unshrunk, non-transparentized fibers crossed by parchmentized cotton yarns which are transparentized throughout the full length thereof. Where both shrinking and parchmentizing processes have been employed successively, fabrics may be produced including shrunk, non-transparentized cellulose fibers crossed by yarns of cellulose fibers which are transparentized throughout the full length of the yarns, the fabric showing a wave effect.

The above statement applies more particularly to an overall treatment with the swelling agents, namely, the shrinking agent or parchmentizing agent. If either of these agents or both agents are applied locally by printing, then the shrunk or

parchmentized yarns may not be swollen throughout their full length but may be partially shrunk or parchmentized in accordance with the printed pattern.

- 5 The term "coated fibres" as employed in the claims is intended to refer to natural fibers containing their natural incrustations, or to natural or artificial fibers which have been coated with one or more of the coating substances herein described, namely, waxes, rubber, chlorinated rubber, hydrocarbons, high boiling fats, varnishes, resins, gums, cellulose ethers and esters, or their equivalents.

- 15 The expression "cellulose fibers" as herein employed is intended to refer to fibers of cotton or other natural cellulose containing fiber or to artificial silks of regenerated cellulose.

- 20 While the invention has been described in detail according to the preferred manner of carrying out the process, it will be obvious to those skilled in the art after understanding the invention, that changes and modifications may be made therein without departing from the spirit or scope of the invention, and it is intended in the 25 appended claims to cover all such changes and modifications.

What is claimed as new and desired to be secured by Letters Patent is:

1. A process for producing pattern fabrics 30 which comprises taking for subsequent treatment a fabric containing inactive and active fibers woven in a pattern, the inactive fibers being coated fibers which are substantially inactive to swelling agents, the active fibers being natural vegetable fibers which have been treated to remove surface incrustations and render the fibers substantially active to swelling agents and treating such fabric with a swell agent to form a visible pattern by altering the active fibers under the swelling action, while the inactive fibers are substantially unaltered thereby.

2. A process for producing pattern fabrics which comprises weaving a fabric according to a pattern using at least two different kinds of yarn, 45 one kind being of inactive coated fibers substantially inactive to agents for opening up the fibers as well as to swelling agents, the other kind of yarn being of natural vegetable fibers retaining their incrustations, treating the fabric to open up the natural vegetable fibers and to render them active to swelling agents and treating such fabric with a swelling agent to form a visible pattern by altering the active fibers under the swelling action while the inactive fibers are substantially unaltered by the opening up and swelling agents.

3. A process for producing pattern fabrics which comprises taking for subsequent treatment a fabric containing inactive fibers and active fibers woven in a pattern, the inactive fibers being substantially inactive to swelling agents and composed of natural vegetable fibers containing their incrustations, the active fibers being natural vegetable fibers which have been treated to remove certain incrustations and render the fibers substantially active to swelling agents, and treating such fabric with caustic soda for shrinking the active fibers to produce a creping effect, the inactive fibers being substantially unaffected by the agent used.

4. A process for producing pattern fabrics which comprises taking for subsequent treatment a fabric containing inactive coated fibers and active fibers woven in a pattern, the inactive fibers being substantially inactive to swelling agents, the

active fibers being natural vegetable fibers which have been treated to remove surface incrustations and render the fibers substantially active to swelling agents, and treating such fabric with sulphuric acid for transparentizing the active fibers, the inactive fibers being substantially unaffected by the agent used.

5. A process according to claim 1 in which after subjecting the fabric to a swelling agent to obtain the desired characteristic effect, the fabric is dyed with a dye which affects the active and inactive fibers differently, thus producing an optical contrast in the dyed fabric due to the different effects of the dye on the active and inactive fibers.

6. A process according to claim 1 in which prior to the application of the swelling agent one or more resist patterns are printed on the fabric.

7. A process for producing pattern effects which comprises taking a fabric of cotton yarn having its natural incrustations and effect yarns of rubber coated yarn, which is inactive to swelling agents, scouring and bleaching the fabric to remove said incrustations and opening up the cotton fibers to render them active and then treating the fabric with a swelling agent to produce shrinkage of the opened-up fibers, the effect yarns being substantially unaffected by the swelling agent.

8. A process for producing pattern effects which comprises taking a fabric of cotton yarn having its natural incrustations and effect yarns of rubber coated yarn, which is inactive to parch-

mentizing agents, scouring and bleaching the fabric to remove said incrustations and opening up the cotton fibers to render them active and then treating the fabric with a parchmentizing agent to produce transparentization of the opened-up fibers, the effect yarns being substantially unaffected by the parchmentizing agent.

9. A process for producing pattern fabrics which comprises taking for subsequent treatment a fabric containing inactive and active fibers woven in a pattern, the inactive fibers being coated fibers which are substantially inactive to swelling agents and the active fibers being natural vegetable fibers which are affected by swelling agents, treating said fabric with a swelling, parchmentizing agent to parchmentize the active fibers, removing the coating from the coated fibers and then treating the fabric with a swelling, shrinking agent to effect shrinking of the now uncoated non-parchmentized fibers.

10. A patterned material formed from fabric containing inactive and active fibers woven in a pattern, the inactive fibers being coated fibers substantially inactive to swelling agents, the active fibers being natural vegetable fibers treated to remove surface incrustations and to render the fibers substantially active to swelling agents, the fabric being treated with a swelling agent to form a visible pattern by altering the active fibers through swelling while the inactive fibers are substantially unaltered thereby.

GEORGES HEBERLEIN.  
ERNST WEISS.

CERTIFICATE OF CORRECTION.

Patent No. 2,275,851.

March 10, 1942.

GEORGES HEBERLEIN, ET AL.

It is hereby certified that error appears in the printed specification of the above numbered patent requiring correction as follows: Page 1, first column, line 18, strike out "or inactive" and insert the same after "insensitive" in line 17; line 45, for "nautral" read --natural--; line 52, for "as not" read --are not--; page 3, first column, line 52, for "this" read --said--; and second column, line 2, after the word "in" insert --the--; page 4, second column, line 38, claim 1, for "swell" read --swelling--; and that the said Letters Patent should be read with this correction therein that the same may conform to the record of the case in the Patent Office.

Signed and sealed this 5th day of May, A. D. 1942.

(Seal)

Henry Van Arsdale,  
Acting Commissioner of Patents.